

## 1

3,401,005

## GERMICIDAL MATERIAL PRODUCED BY MODIFYING TEXTILE FIBERS WITH A METHYLOLATED LACTAM AND TREATING SAME WITH IODINE

Leon Katz, Springfield, N.J., assignor to GAF Corporation, a corporation of Delaware  
No Drawing. Filed Oct. 22, 1965, Ser. No. 502,618  
6 Claims. (Cl. 8—115.5)

The present invention relates to novel germicidal products suitable for use as bandages, surgical dressings and the like.

In the copending application of Randall and Freyermuth, Ser. No. 502,387, filed Oct. 22, 1965, there is disclosed fibrous materials treated with N-hydroxymethyl lactams such as N-hydroxymethylpyrrolidinone. I have discovered that when the thus treated fibrous material is further treated with a halogen containing germicidal agent such as iodine, iodine monochloride or iodine monobromide, the germicidal agent combines with the treated fibrous material in an effective amount so as to produce a germicidal fibrous material suitable for the production of bandages and surgical dressings and the like in which the germicidal activity is retained for substantial periods of time.

The novel germicidal fibrous materials of the present invention are readily prepared by directly applying to the treated fibers, more fully described and claimed in aforementioned application of Randall and Freyermuth, a halogen containing germicidal agent. The germicidal agent can be applied directly to the treated fibers or preferably a solution thereof is applied to the treated fibers. The germicidal agent combines with the treated fibers and renders the fibers germicidally effective for substantial periods of time. The combination of the germicidal agent with the treated fibers can be affected by prolonged contact at ordinary temperatures or preferably may be expedited by the use of elevated temperatures during or immediately following application of the germicidal agent to the treated fibers.

The details of the present invention will be apparent to those skilled in the art from a consideration of the following specific examples of preferred embodiments thereof.

### EXAMPLE A

#### Preparation of treated fibers

An aqueous solution containing 10% N-hydroxymethylpyrrolidinone and 0.36%, 2-methyl-2-amino-1-propanol hydrochloride was padded on cotton gauze (hospital bandage material). The gauze, padded with N-hydroxymethyl pyrrolidinone, was squeezed through rubber rollers with sufficient pressure to give 100% (by weight) wet pick-up of solution. The fabric in roll form was dried at about 100° C. and then heat cured at 150–155° C. for three minutes. The roll of gauze was rinsed with warm water on a laboratory jig, squeezed between pressure rollers, and dried. The cloth after this treatment contained 0.61% nitrogen. This indicated that 50.0% of the total amount used of the N-hydroxymethylpyrrolidinone had reacted, to yield cotton gauze, containing 5% by weight chemically reacted N-hydroxymethylpyrrolidinone.

In a similar manner a rayon gauze, hospital bandage material, was treated with 10% N-hydroxymethylpyrrolidinone and it was found that the rayon material, after this treatment, contained 0.36% of nitrogen indicating that 30% of the total amount used of the N-hydroxymethylpyrrolidinone had reacted to yield rayon gauze containing a 3% by weight chemically reacted ethylhydroxymethylpyrrolidinone.

## 2

### EXAMPLE 1.

Three square pieces of cotton fabric each weighing 7.3 g. which had been treated with N-hydroxymethylpyrrolidinone in the manner described above, were rolled up and placed in a wide mouth bottle 6.5 inches high and 2.5 inches in diameter in such a manner that the outer surface of cloth bands touched the surrounding inner curved surface of the bottle. In the center of the roll of the cotton was carefully inserted an inverted 50 ml. beaker, and 10 ml. beaker containing 0.73 g. iodine crystals was placed on the inverted beaker. The bottles were then tightly capped and sealed with a sheet of polyethylene under the cap. The bottles were allowed to stand at room temperature for two weeks during which time the iodine sublimed and reacted with the cloth giving it a reddish-brown color similar in shade to that of the polyvinylpyrrolidinone iodine complex described in U.S. Patent N. 2,739,922. The treated cloth was then removed from the bottle, rinsed with cold water and dried. It was found to contain 7.5% iodine by analysis.

The thus treated cotton cloth was then evaluated for germicidal activity, along with the following control samples of cotton fabric.

Sample A: 80 x 80 untreated cotton fabric (no treatment with N-hydroxymethylpyrrolidinone) but treated with iodine in the manner described above.

Sample B: 80 x 80 cotton fabric treated as described above with N-hydroxymethylpyrrolidinone and then treated with iodine as described above.

This germicidal activity evaluation was conducted by both a use dilution test and a zone of inhibition test. The procedures of these tests were as follows:

#### Use dilution test

35 Ten 2 x 2 cm. swatches of each of the treated cloths were placed in sterile petri dishes. 0.1 cc. of 1:1,000 dilution of a 24 hours broth culture of *S. aureus* ATCC6538 was placed on each swatch and the petri dishes then placed in an incubator at 37° C. for 15 minutes. At the 40 end of the 15 minutes contact time, the inoculated swatches of cloth were removed to tubes containing 10 cc. of FDA broth using sterile forceps and these tubes incubated at 37° C. for 24 hours at which time they were recorded as positive or negative from the standpoint of 45 turbidity.

To eliminate the possibility of turbidity due to the bacteriocidal agent on the cloth or the possibility of an apparent negative result being bacteriostatic rather than a bacteriocidal effect, transfers of 0.1 cc. were made to new FDA broth tubes from the 24 hour tubes which contained the cloth. These transfers were incubated for an additional 24 hours at 37° C. at which time the final readings were taken from both sets of tubes.

#### Zone of inhibition test

55 Ten 2 x 2 cm. swatches from each cloth were placed on FDA agar plates (one swatch/petri dish) and were overlayed with 100 cc. of FDA agar inoculated with 0.1 cc. of a 1:1,000 dilution of a 24 hour broth culture of *S. aureus* ATCC6538. The plates were allowed to harden, and then incubated at 37° C. for 24 hours at which time the zone of inhibition around each swatch was determined.

65 The results were as follows:

#### USE DILUTION TEST

|                  | Number of tubes negative out of 10 |           |
|------------------|------------------------------------|-----------|
|                  | Initial                            | Transfers |
| 70 Sample A..... | 10                                 | 10        |
| Sample B.....    | 10                                 | 10        |

Zone of inhibition, average zone size:

Sample A, trace  
Sample B, 3-4 mm.

Conclusions: As tested, both materials exhibit the same degree of bacteriocidal action in the broth system. However, in the agar system, Cloth B exhibits a much greater bacteriocidal action than Cloth A.

### EXAMPLE 2

8.70 g. samples of both the cotton gauze material and the rayon gauze material prepared as described above in Example A, were rolled up and placed in 16 oz. wide mouth glass bottles, approximately 6.5 inches high and 2.5 inches in diameter in such a manner that the outer surface of a gauze band touched the surrounding inner curved surface of the bottle; in the center of each of the rolls of gauze was carefully enclosed 10 ml. beaker on top of which was placed a 5 ml. beaker containing iodine crystals. The bottles were then tightly capped and sealed with a small sheet of polyethylene under the cap, and the bottles and their contents were placed in an electric oven and heated to 90° C. for 4 hours. After cooling to room temperatures, the germicidal bandage material was removed from the bottles and hung on a line in the atmosphere for one hour before beginning stability tests. The percent by weight of iodine, based on the weight of the gauze material, contained in the 5 ml. beaker and also the percent by weight of elemental iodine and HI as determined by analysis to be present in the gauze, both initially and after storage and is given in the following Table I.

TABLE I

| Material                                                     | Sample |       |
|--------------------------------------------------------------|--------|-------|
|                                                              | 1      | 2     |
|                                                              | Cotton | Rayon |
| Percent Iodine in 5 ml. Beaker                               | 0.50   | 0.50  |
| Percent HI Found (initially)                                 | 0.06   | 0.05  |
| Percent I <sub>2</sub>                                       | 2.25   | 0.10  |
| Percent HI—after 9 days at 40° C. open bottle                | 0.29   | 0.14  |
| Percent I <sub>2</sub> —after 9 days at 40° C. open bottle   | 0.20   | 0.09  |
| Percent HI—after 20 days at 40° C. open bottle               | 0.22   | 0.16  |
| Percent I <sub>2</sub> —after 20 days at 40° C. open bottle  | 0.19   | 0.07  |
| Percent HI—after 9 days at 25° C. sealed bottle              | 0.76   | 0.16  |
| Percent I <sub>2</sub> —after 9 days at 25° C. sealed bottle | 0.26   | 0.09  |

### EXAMPLE 3

2.5 g. iodine crystals were dissolved in 250 ml. solvent at room temperature with stirring. Cotton gauze (from Example A) was padded with the aforementioned tincture of iodine and squeezed through rubber pressure rollers so that the wet pick-up by the gauze was 66% (by weight). The padded gauze was dried in air at room temperature for 15 minutes and then was given one of the following treatments:

- (A) Heat cured for 3 minutes at 150° C. in an oven.
- (B) Heat cured in a sealed container at 90° C. for 4 hours.
- (C) Heat cured in an open vessel at 90° C. for 4 hours.

The analytical results are indicated on the attached Table II.

iodine monobromide will also combine with the N-hydroxymethylpyrrolidinone treated fibers and to be retained thereby for a substantial period of time so as to produce a germicidally active fibrous material substantially free of irritating or sensitizing characteristics frequently found in the germicidal agent itself or when present on other substrate.

It will also be understood that while fibrous material treated with N-hydroxymethylpyrrolidinone was employed in the foregoing examples and represents a preferred form of fibrous material for use in the practice of the present invention that fibrous materials treated with other N-hydroxymethyl lactams or ethers thereof, more fully described in the above mentioned invention of Randall and Freyermuth, Ser. No. 502,387, Oct. 22, 1965, may be used in practicing in the present invention. Thus, there may be used cellulosic materials treated as described in said application with an N-hydroxymethyl lactam of the formula



and ring carbon-lower alkyl substituted derivatives thereof, wherein R represents an alkylene bridge such as, for example, ethylene, propylene, butylene, necessary to complete a 5 to 7 membered heterocyclic ring; and R' represents hydrogen or lower alkyl such as methyl, ethyl, propyl, isopropyl, butyl, isobutyl, and the like. As examples of such N-hydroxymethyl lactams may be mentioned, in addition to N-hydroxymethylpyrrolidinone, the following.

#### Pyrrolidones:

- N-methoxymethyl pyrrolidinone-2
- 3,3-dimethyl-N-hydroxymethylpyrrolidinone-2
- 3,3,5-trimethyl-N-hydroxymethylpyrrolidinone-2
- 3,3,5-trimethyl-N-methoxymethylpyrrolidinone-2
- 3-propyl-5-methyl-N-hydroxymethylpyrrolidinone-2

#### Piperidones:

- N-hydroxymethylpiperidone-2
- N-methoxymethylpiperidone-2
- 4,4-dimethyl-N-hydroxymethylpiperidone-2
- 6-propyl-N-methoxymethylpiperidone-2
- 4,4-dimethyl-N-ethoxymethylpiperidone-2

#### Epsilon-caprolactams:

- 3,3,5-trimethyl-N-hydroxymethyl-E-caprolactam
- N-hydroxymethyl-E-caprolactam
- N-methoxymethyl-E-caprolactam
- 4,4-dimethyl-N-ethoxymethyl-E-caprolactam

The N-hydroxymethyl lactam treated fibrous material, employed in practicing the present invention, preferably contains about 5% by weight of the N-hydroxymethyl lactam combined with the fibers. However, the N-hydroxymethyl lactam treated fibrous materials have the property of combining with halogen containing germicidal agents when the N-hydroxymethyl oxide content thereof is varied over relatively wide ranges, and effective products have been produced using fibrous materials having

TABLE II

| Sample | Heat curing treatment | Solvent                   | Wt. percent I <sub>2</sub> in solvent | Wt. percent in pick-up by cloth | Wt. percent I <sub>2</sub> on cloth before curing treatment | Wt. percent I <sub>2</sub> retained by cloth after curing treatment | Wt. percent HI on cloth after curing treatment |
|--------|-----------------------|---------------------------|---------------------------------------|---------------------------------|-------------------------------------------------------------|---------------------------------------------------------------------|------------------------------------------------|
| 1..... | A                     | Ethanol.....              | 1.23                                  | 65.8                            | 0.81                                                        | 0.28                                                                | 0.59                                           |
| 2..... | B                     | do.....                   | 1.23                                  | 65.8                            | 0.81                                                        | 0.36                                                                | 0.86                                           |
| 3..... | C                     | do.....                   | 1.23                                  | 92.6                            | 1.14                                                        | 0.70                                                                | 0.27                                           |
| 4..... | A                     | Carbon tetrachloride..... | 0.62                                  | 74.0                            | 0.46                                                        | 0.01                                                                | 0.23                                           |
| 5..... | B                     | do.....                   | 0.62                                  | 74.0                            | 0.46                                                        | 0.42                                                                | 0.10                                           |
| 6..... | C                     | do.....                   | 0.62                                  | 159.0                           | 0.99                                                        | 0.62                                                                | 0.07                                           |

While iodine was employed in the foregoing examples as a preferred germicidal agent, it should be understood that the interhalogen adducts, iodine monochloride and

combined therewith from about 2% to 10% by weight of N-hydroxymethyl lactam. Likewise, the amount of halogen containing germicidal agent employed in practic-

ing the present invention may be varied at relatively wide ranges. About 0.5% of the germicidal agent by weight is preferred but products containing as low as 0.1% of germicidal agents, have been found to be effective. The maximum amount of germicidal agent which can be combined with the N-hydroxymethyl fibrous treated material will vary substantially directly with the amount of N-hydroxymethyl lactam combined with the fibrous material. An amount of germicidal agent corresponding to 10% of the amount of N-hydroxymethyl lactam combined with the fibrous material can readily be incorporated in the products as illustrated by the foregoing examples. Larger amounts of up to 20 to 25% by weight of the N-hydroxymethyl lactam have, however, been successfully incorporated in the final products.

What is claimed is:

1. A process for producing germicidal fibrous materials which comprises applying a halogen containing germicidal agent selected from the group consisting of iodine, iodine monochloride and iodine monobromide to 20 cellulosic fibrous material obtained by reacting a lactam derivative of the formula

(I)



25

and ring carbon-lower alkyl substituted derivatives thereof, and wherein R represents a lower alkylene group necessary to complete a 5 to 7 membered heterocycle and R' is selected from the group consisting of hydrogen and lower alkyl, and then drying and curing the fibrous material at a temperature of at least about 120° C.

- 5 2. A process as defined in claim 1 wherein the lactam is N-hydroxymethylpyrrolidinone-2.
- 10 3. A process as defined in claim 2 wherein the germicidal agent is iodine.
- 15 4. A process as defined in claim 3 wherein the fibrous material is heated to a temperature of about 90° C. following the application of iodine thereto.
- 5 5. A germicidal fibrous material produced according to the process in claim 1.
- 15 6. A germicidal fibrous material produced according to the process in claim 4.

#### References Cited

##### UNITED STATES PATENTS

3,136,755 6/1964 Grosser et al. \_\_\_\_\_ 167—38.6 X

##### FOREIGN PATENTS

1,070,588 12/1959 Germany.

NORMAN G. TORCHIN, *Primary Examiner.*

J. C. CANNON, *Assistant Examiner.*